

Dec. 15, 1959

R. E. COFFEE

2,916,996

PROPELLENT POWDER

Filed Feb. 29, 1956

FIG. 1



FIG. 2



INVENTOR.  
RALPH E. COFFEE  
BY *John D. Sonnenburg*  
*Leonard D. Goff*  
ATTORNEYS

1

2,916,996

## PROPELLENT POWDER

Ralph E. Coffee, Berkeley, Mo., assignor to Olin Mathieson Chemical Corporation, East Alton, Ill., a corporation of Virginia

Application February 29, 1956, Serial No. 568,945

4 Claims. (Cl. 102—98)

This invention relates generally to explosives and more particularly to smokeless powder having improved burning characteristics.

It has been proposed heretofore to provide high energy smokeless powder by embedding particles of a solid high explosive in a matrix of a smokeless powder base such as nitrocellulose or a mixture of nitrocellulose and nitroglycerine. U.S. 2,425,854 discloses a propellant powder of this type having the particles of high explosive dispersed substantially uniformly throughout the powder grain. The ballistic characteristics of such powders are an improvement over double base high energy powders depending upon large quantities of nitroglycerine mixed with the nitrocellulose to impart the high energy characteristic, but they have the objectionable feature of developing high breech pressures when loaded in cartridges in quantities sufficient to impart high velocities to the projectile. Moreover, as pointed out in the above referred to patent, it is impossible to coat such powder grains satisfactorily with a deterrent to impart maximum progressive burning characteristics to the grain.

It is, therefore, an object of this invention to provide a smokeless powder adapted to burn progressively and impart high velocities to projectiles at improved breech pressure levels. Another object of the invention is to provide a novel smokeless powder having improved burning characteristics which impart high velocities to projectiles with less breech pressure than the heretofore available powders. Still another object of the invention is to provide a high energy smokeless powder containing particles of a solid high explosive having a deterrent coating on the surface thereof. Still another object of the invention is to provide a smokeless powder containing particles of a solid high explosive having an improved gravimetric density. A more specific object of the invention is to provide a smokeless powder grain having a nitrocellulose matrix with particles of a solid high explosive embedded therein having improved progressive burning characteristics.

The foregoing objects as well as others are accomplished in accordance with this invention, generally speaking, by providing a progressive burning powder having a core containing particles of a solid high explosive substantially uniformly dispersed in a smokeless powder base matrix, and an envelope of smokeless powder base surrounding the core which contains a lesser percentage by weight of high explosive or is substantially devoid of high explosive particles. The smokeless powder base matrix may be composed of gelatinized nitrocellulose or gelatinized nitrocellulose mixed with nitroglycerine or any other suitable nitric ester of a polyhydric alcohol, such as for example, dinitroglycol.

The powder grains may be formed in the first step of the process by any conventional method suitable for forming grains having particles of solid high explosives dispersed in a smokeless powder base matrix. Globular powder grains of high density may be formed by a process similar to that disclosed by Schaefer in U.S. Patent 2,160,626 modified to the extent that solid particles of high explosives are suspended in the lacquer globule before it is hardened by removing the solvent. The grains having the particles of high explosive dis-

2

persed throughout their structure are then extracted with a suitable solvent for the smokeless powder matrix to erase the pits left in the surface by the removal of the particles of high explosive and to produce a grain having a substantially smooth surface. The grain may be coated with a suitable deterrent, if desired, to further improve the progressive burning characteristics of the grain.

Any secondary solid explosive which is incompletely soluble in the other ingredients of the powder grain and develops greater energy upon burning than nitrocellulose may be utilized. Examples of such explosives are pentaerythritol, tetranitrate, trinitrotoluene, cyclonite (cyclotrimethylenetrinitramine), homocyclonite (cyclo-tetramethylenetrinitrate), tetryl and the like. Of these explosives, cyclonite is preferred because of the pressure velocity relationship obtained with smokeless powders containing this material.

The solid high explosive may be extracted either with any suitable solvent for the high explosive which is also a solvent for the smokeless powder base matrix or with any suitable solvent for the high explosive which is not a solvent for the smokeless powder base. Examples of solvents which fall in the latter category are ethyl alcohol, xylene, benzene, toluene, methyl alcohol, isopropyl alcohol, isobutyl alcohol and the like. Solvents suitable for the purpose which dissolve both the smokeless powder base and the solid high explosive particles include acetone, dimethylformamide, cyclohexanone and the like.

In a preferred form of the invention, the powder grains having the particles of solid high explosive dispersed substantially throughout the grain are suspended in a suitable non-solvent for the powder grains such as water having dissolved therein sufficient solvent to extract all of the solid high explosive from the outer shell of the grain and the slurry is agitated until the particles of high explosive have been extracted therefrom. The thickness of the envelope or outer shell from which the solid high explosive is extracted may be varied somewhat depending upon the particular ballistic characteristics desired but it should not be more than about  $\frac{1}{4}$  of the diameter or thickness of the grain to provide a grain having high energy characteristics with attending low pressure characteristics.

It has been found that cartridges containing a propellant charge of the powder provided by this invention impart a much higher muzzle velocity to the projectile at lower breech pressures than cartridges having a propellant charge of smokeless powder having the particles of high explosive dispersed substantially uniformly throughout the grain including the outer shell. Moreover, by treating the powder grains after the high explosive has been extracted from the outer shell thereof with a suitable solvent for the smokeless powder base, such as for example, ethyl acetate, methyl ethyl ketone and the like to case harden the surface of the grains and to provide a substantially smooth surface without any pits therein, the gravimetric density of the powder grain is greater than that obtainable with powder grains having the high explosive distributed throughout the grain. For example, propellants having a gravimetric density as high as 1.000 have been prepared in accordance with this invention whereas the maximum density heretofore obtained with powders of the other type containing an equivalent amount of solid high explosive per unit of weight has not been greater than about 0.940. The solid particles of high explosives do not migrate into the outer shell even during long storage periods at elevated temperatures so the powder is more ballistically stable than powders depending upon nitroglycerine for their high energy characteristics.

In order better to describe and further clarify the invention, the following are detailed descriptions of preferred embodiments thereof taken in connection with the drawing in which:

Figure 1 is a flow diagram illustrating the steps of the process of the present invention; and

Figure 2 is a cross-sectional view of a powder grain resulting from the process.

The process of the present invention can be carried out in conventional grain forming and treating apparatus. The grains are formed from a mixture of a propellant powder base and a solid high explosive in any desired manner in standard grain forming apparatus 1. If the process employed involves suspension in a non-solvent medium, the powder grains are filtered from the liquid medium as indicated at 2 and the high explosive material at or near the surface of the grain is extracted as indicated at 3 with a solvent therefor carried in an aqueous medium. After the surface extraction of the high explosive from the powder grains, they are separated from the liquid medium by filtration 4 or other suitable means and then suspended in an aqueous medium containing a solvent for the smokeless powder base. This treatment is continued until the grains are provided with a smooth imperforate surface layer of the powder base. The surface hardening step is indicated generally at 5. The grains which have thus been extracted and surface hardened are then separated from the suspending medium and subsequently dried.

*Example 1*

About 75 parts by weight nitrocellulose having a nitrogen content of about 13.2 percent are added to about 1500 parts water in a suitable grain forming still indicated generally at 1 at a temperature of about 50° C. and the resulting slurry is agitated to suspend the nitrocellulose therein. About 94 parts by weight cyclonite are suspended in about 375 parts ethyl acetate having dissolved therein about 0.75 part diphenylamine as a stabilizer. This mixture is agitated to suspend the cyclonite therein and the suspension is then added to the nitrocellulose-water slurry. The resulting slurry is agitated as it is heated to about 68° C. After the nitrocellulose has dissolved, about 3 parts of a protective colloid derived from animal protein or an equivalent amount of gum arabic or any other suitable protective colloid are added and the slurry is agitated until the lacquer formed by the dissolution of the nitrocellulose is broken up into globules of the desired particle size. About 40 parts sodium sulfate dissolved in about 200 parts water are added to the slurry and agitation of the slurry is continued for about three hours while the temperature is gradually raised to about 99° C. to remove the ethyl acetate and convert the globules of lacquer into hardened powder grains having cyclonite distributed substantially uniformly throughout each grain. The composition of such grains is about 55 percent cyclonite, about 44.5 percent nitrocellulose and about 0.5 percent diphenylamine. These grains are separated from the liquid medium by filtering or other suitable means as indicated at 2 in the drawing.

In order to remove a total of about 15 percent of the cyclonite from the powder grain and to limit the removal to the outer shell of the grain, about 200 parts by weight of the powder grains prepared above are agitated in about 1260 parts ethyl alcohol, at about 76° C. in a slitable vessel 3 until the alcohol is saturated with cyclonite. The resulting powder grains will contain about 42.5 percent cyclonite and all of this cyclonite will be in the core of the grain with the outer shell of the grain being substantially devoid of any particle of cyclonite.

If desired, the foregoing extraction process may be modified by using amounts of solvent, such as ethyl al-

cohol, greater than that which will become saturated with the amount of cyclonite desired to be removed from the grain and to control the time in which the grains are exposed to the solvent action in order to control the amount of cyclonite removed therefrom. The cyclonite may be recovered from the ethyl alcohol or other liquid used for the extraction thereof by any suitable means.

*Example 2*

In another embodiment of the invention, powder grains shaped in accordance with the process disclosed above and containing particles of cyclonite distributed substantially uniformly throughout the structure are extracted with acetone which is a solvent for the nitrocellulose as well as for the cyclonite. About 100 parts of the powder grains are agitated in a solution of about 395 parts acetone and about 495 parts water for about 15 minutes at about 55° C. The powder grains are then separated from the liquid phase by filtration or other suitable means 4 and washed with water to remove the last traces of the suspending liquid.

The powder grains extracted by either of the foregoing processes are surface hardened as indicated at 5 by suspending them in a water medium having a solvent phase. About 100 parts by weight of the powder grains are suspended in about 400 parts water containing about 5 parts gum arabic. About 75 parts ethyl acetate are added to the suspension and the slurry is agitated while the temperature is increased to about 70° C. A salt solution may be added at this point to help improve gravimetric and grain density in accordance with the process disclosed by Schaefer in U.S. 2,160,626. Agitation is continued at this temperature for about two hours after which time the surface of the powder grains will have been softened by the solvent, lost the pits therein and assumed a substantially smooth surface. The temperature is gradually elevated to about 99° C. to remove the ethyl acetate. The grains are then separated from the liquid by filtering or other suitable means. The gravimetric density of the grains is increased by this treatment. Grains having a gravimetric density of about 0.920 before extraction have a gravimetric density of about 1.000 after extraction of the cyclonite and after surface treatment of the grains in accordance with this procedure.

The grains obtained in accordance with the present invention are well illustrated in Figure 2 of the drawing. As indicated, the grains are substantially non-porous and consist of a central core portion 6 throughout which discrete particles 7 of a high explosive material, such as cyclonite, are uniformly dispersed. The core portion of the grain is completely encased in a surrounding envelope 8 which is substantially smooth and imperforate and also free of significant amounts of the secondary explosive.

As an example of the improved ballistic properties of propellant grains formed in accordance with this process, powder grains have a diameter of between 0.025 inch and 0.034 inch containing about 50 percent cyclonite substantially uniformly dispersed therein were loaded in conventional caliber .50 cartridge cases and fired in caliber .50 machine guns. Similar cartridges were then loaded with powder prepared in accordance with this invention by extracting the nitrocellulose base powder grains containing 50 percent cyclonite with ethyl alcohol to remove all of the cyclonite from the outer shell until the total amount of cyclonite in the grain was reduced to about 40 percent cyclonite. The following results were obtained:

|                           | Charge<br>(grains) | Pressure<br>(p.s.i.) | Velocity<br>(ft./sec.) |
|---------------------------|--------------------|----------------------|------------------------|
| 40% Cyclonite Powder----- | 145                | 51,700               | 2,634                  |
| 50% Cyclonite Powder----- | 145                | 53,700               | 2,682                  |

These data show that a charge of a nitrocellulose base powder provided by this invention containing 40 percent cyclonite propelled the projectile at a muzzle velocity greater than the muzzle velocity of the projectile propelled by the powders having 50 percent cyclonite dispersed substantially uniformly therein and at a breech pressure of 2000 pounds per square inch less than the breech pressure developed by the powder containing the 50 percent cyclonite. A similar improvement is obtained in accordance with this invention with propellents containing one of the other secondary solid explosives set forth hereinbefore and also with propellant grains containing particles of nitroguanidine.

As indicated hereinbefore the powder grains can be made by any suitable process and then extracted in accordance with this invention. For example, any suitable extrusion or casting process for shaping propellant grains containing a solid high explosive dispersed in discrete form therein can be utilized. In making powder in accordance with the preferred embodiment disclosed above, any other suitable non-solvent medium may be utilized in lieu of water and any other suitable solvent may be used instead of ethyl acetate. The solvent should be substantially immiscible with the non-solvent medium. Examples of suitable solvents include methyl ethyl ketone, isopropyl acetate, ethylformamide, methyl isobutyl ketone and the like. The powder grains after the surface treatment to remove the pits therefrom may be treated with a deterrent in accordance with any suitable procedure, such as for example, by the emulsion coating process disclosed by Wagner in U.S. Patent 1,924,967. Suitable deterrents include dibutyl phthalate, diphenyl phthalate, ethyl centralite and the like. The grains may also be coated with nitrocellulose if desired by any suitable procedure including the one disclosed in the Wagner patent U.S. 1,862,914.

Although the invention has been described in detail in connection with the preparation of powders containing

cyclonite, other solid high explosives can be incorporated in powder and extracted in a similar manner, and it is to be understood that the purpose of this detail is solely for illustration and that modifications can be made in the embodiments without departing from the spirit and scope of the invention except as it is limited by the appended claims.

I claim:

- 10 1. A progressive burning smokeless powder grain comprising a core having a matrix of a smokeless powder base containing particles of a solid high explosive distributed substantially uniformly therein, a substantially imperforate envelope enclosing said core of gelatinized smokeless powder base said envelope being substantially devoid of solid high explosive particles and having a substantially smooth, imperforate surface, and on said envelope a coating of a deterrent.
- 15 2. The product of claim 1 wherein said high explosive is pentaerythritol tetranitrate.
- 20 3. The powder grain of claim 1 wherein the core contains at least 15% by weight of the high explosive.
- 25 4. A process for making smokeless powder grains having improved velocity and breech characteristics comprising mixing particles of a solid high explosive with a smokeless powder base, shaping the resulting mass into powder grains, subjecting the resulting grains to the action of a solvent for the high explosive until substantially all of the particles of high explosive in the outer shell of the grains have been dissolved in the solvent and
- 30 35 removed therefrom, and thereafter maintaining the grains in an aqueous suspension of a solvent for the smokeless powder base until the surface of the grains has become substantially smooth.

References Cited in the file of this patent

UNITED STATES PATENTS

- |           |           |               |
|-----------|-----------|---------------|
| 1,906,675 | Wagner    | May 2, 1933   |
| 2,425,854 | Alexander | Aug. 19, 1947 |